

# UNITED STATES PATENT OFFICE.

HUGH RODMAN, OF EDGEWOOD, PENNSYLVANIA, ASSIGNOR TO RODMAN CHEMICAL COMPANY, OF VERONA, PENNSYLVANIA, A CORPORATION OF PENNSYLVANIA.

## CASE-HARDENING MATERIAL.

1,317,728.

Specification of Letters Patent.

Patented Oct. 7, 1919.

No Drawing.

Application filed June 16, 1917. Serial No. 175,236.

*To all whom it may concern:*

Be it known that I, HUGH RODMAN, a citizen of the United States, and a resident of Edgewood, in the county of Allegheny and 5 State of Pennsylvania, have made a new and useful Invention in Case-Hardening Material, of which the following is a specification.

This invention relates to case-hardening 10 and discloses a new and improved case-hardening material and method of using that material.

It is old to use coking coal in making 15 case-hardening material. This is generally done by crushing the coal to a fine powder, mixing with powdered energizing materials, coking the mixture to produce large lumps of impregnated coke and then crushing these 20 lumps and screening to secure smaller lumps of about one-quarter inch in through dimension.

Another method followed on a commercial 25 scale is to mix powdered coking coal and energizing material with binding material and fashion therefrom small masses which will remain as individual small masses when they are heated to a coking or carburizing temperature.

Each of these methods of using coking 30 coal as a base for the manufacture of case-hardening material has been commercially utilized and satisfactory material obtained. It is to be observed, however, that material made by either method, as well as any carburizing material in the form of small 35 lumps (as distinguished from dust) is liable to disintegrate somewhat in service, especially when subjected to repeated re-use, and to make dust, which is not only difficult to 40 handle but also reduces the efficiency of the carburizing material. It is general practice to screen out this dust as formed, entailing loss of material and labor.

I have observed that case-hardening 45 material containing raw, unheated material (raw bone as against charred bone, coal as against coke) are more energetic than the same material after heating, which fact I attribute to the gases evolved at low temperatures 50 when these raw materials are heated with energizing materials in the presence of the steel or iron to be carburized. However, in the use of raw coking coal for this purpose, there is the practically insuperable objection that the coal mixture will coke to a

solid coke, entangling the iron and steel parts and often warping them.

I have found a satisfactory method of overcoming this difficulty, as well as largely overcoming the tendency of carburizing material to form dust in service. This consists in making a mixture of crushed coking coal and energizing material (to which may be added a little oil to lay the dust if desired) and then adding this mixture in the 60 ratio of about one to four to previously used carburizing material. This scheme of adding fresh carburizing material to previously used carburizing material is the ordinary practice in most shops, and is generally 65 done after the used material has been cooled down from its carburizing heat; therefore, the use of this scheme in the process I am describing entails no special effort.

I find that when some of my coking coal 70 mixture is added to previously used material and the resultant mixture is used in carburizing operations the coking coal will coke or frit the previously used material together just enough to insure a tying together of 75 the dust, but not enough to hinder the easy removal of the steel parts and not enough to cause any warping of the steel. In this way I secure several valuable improvements 80 in the carburizing of steel. First, I am enabled to use the very cheap carburizing agent consisting of a mixture of crushed coking coal and energizers. Second, I secure 85 the high efficiency due to the use of raw coal rather than to coke. Third, I overcome the 90 tendency of the carburizing material to form dust. Fourth, I produce a material of high thermal conductivity due, I believe, to the light fritting of the entire mass. Fifth, I overcome the tendency of some materials to 95 stick or adhere to the steel after the material has been used. Sixth, I prevent the shrinkage in volume which most materials undergo when highly heated. The raw coal mixture seems to insure a clean surface even 100 when mixed with used material which would, alone, ruin the surface of the steel parts.

It is apparent that the permissible amount of coal mixture which can be added to the used material will depend upon the nature of the used material and also upon the coking strength of the coal mixture. I find that, using the preferred coal mixture which I will describe later on, and adding this to carburizing material which has been secured 110

through previous repeated additions of coal mixture, about twenty to thirty per cent. of coal mixture will give excellent results. In other words, I maintain a constant supply 5 of highly efficient carburizing material, as well as largely overcome the formation of dust, by adding about twenty-five per cent. of the coal mixture to the used material each time it has been cooled down after a car- 10 burizing heat. I find that this may be conveniently done by shoveling the two materials together, as concrete is mixed, on the floor, but special mixing devices can, of course, be used if desired.

15 The coal mixture can be varied within wide limits and still insure excellent results, but I have found the following to give satisfactory results and prefer it because of its cheapness and large supply. I crush a good 20 grade of Pittsburgh seam coking coal so it will pass a screen having eight wires to the linear inch and mix with this twelve and one-half per cent. of powdered soda ash (sodium carbonate) and twenty parts of calcium carbonate, each by weight. To this 25 mixture I then add ten per cent. (based upon the weight of the coal) of fuel oil so as to lay the dust. I find that this amount of oil will also be enough to lay the dust of the 30 mixture when this coal mixture is later mixed with the used material. Other proportions of energizer and coal may be used, and other energizers such as barium carbonate may be used.

35 In adding the coal mixture to the used material for the first time it is necessary to use some care, as less coal mixture can be added to large size granular material than to material consisting largely of small particles 40 and dust. If too much coal mixture is used the mass of mixed material will fit together more solidly than is desired;—and of course, if the coal mixture is used alone it will coke to a solid coke, firmly embedding 45 the metal parts and probably warping them. Where it is necessary to begin carburizing operations without a supply of used material, I prefer to start with material having a coke base (though other materials may be 50 used) and to screen this so it will pass through a screen having about ten wires to the linear inch and to remove all or most of the fine dust. When the coal mixture is added to this in the proportion of about 55 twenty-five per cent., and this addition is thereafter made following each carburizing heat, there is maintained a carburizing material of exceptionally high efficiency, low cost and with such desirable characteristics 60 as high thermal conductivity, freedom from dust, low volumetric shrinkage, ability to produce clean steel surfaces, etc.

I have used this system of adding a coking 65 coal mixture to previously used carburizing material successfully and on a large scale and I believe I am the first to do so, or to propose its use in this way. It is likely that other strongly coking materials, as an asphaltum and energizer mixture might be used in the same way. It is no doubt pos- 70 sible to make small masses of mixed pitch and energizer, such as would, if heated alone, go down into a solid coke, and yet which would, if mixed with previously used carburizing material in proper proportions, frit 75 or coke the used material to a light and desirable amount and bind the dust as already described. Such materials, would I believe, come within the scope of this invention, and they may be termed strongly coking ma- 80 terial, since they like the Pittsburgh seam coking coal, are characterized by the fact that in coking they form a solid structure of considerable mechanical strength. In addition to this, the "strongly coking" quality of 85 these materials is such as to cause them when mixed with separate particles of other non-coking materials, to form a solid or coke like structure when heated to a coking temperature, but, as stated, I prefer to use ordi- 90 nary coking coal because of its cheapness and availability and because I have thoroughly demonstrated its practicability.

It is obvious that the same end could be secured by maintaining sufficient energizer 95 in the used material, adding more from time to time as needed, and then add the coking coal or coking material only, but this is not so satisfactory as the method described and would be only another way of getting at the 100 same object.

What I claim is :

1. The method of revivifying spent carburizing material which consists in intimately mixing previously used carburizing 105 material with strongly coking material capable of fritting the mass of previously used material together to form a coke like structure when subjected to a coking temperature.
2. The method of carburizing steel which consists in heating the steel part to be carburized to a carburizing temperature in a mixture of previously used carburizing material and a coking material capable of fritting the mixture together to form a coke like structure when subjected to the carburizing temperature.
3. The method of revivifying spent carburizing material which consists in intimately 120 mixing spent carburizing material with an energizer and a coking material capable of fritting the separate particles of the mass together to form a coke like structure when heated to a carburizing temperature.
4. The method of carburizing steel and revivifying spent carburizing material which consists in packing the steel to be carburized in an approximately homogeneous mixture of finely divided spent carburizing material 130

and finely divided strongly coking material capable of fritting the separate particles of the mixture together to form a coke like structure, and then in subjecting the mixture

5 and the steel to a carburizing heat.

5. Carburizing material comprising a mixture of finely divided previously used carburizing material and crushed coking coal in the proportions of approximately

10 three parts of used material to one part of coal.

6. A carburizing material comprising a mixture of about three parts of previously used carburizing material, and one part

15 crushed coking coal, and an energizer.

7. The method of carburizing steel which consists in heating it in a mixture of previously used carburizing material and a strongly coking material containing coking

20 coal.

8. The method of carburizing steel which

consists in heating it in a mixture of previously used carburizing material and a strongly coking mixture of coking coal and an energizer.

25

9. The method of carburizing steel which consists in heating it in a mixture of previously used carburizing material and a strongly coking mixture containing coking coal, soda ash and calcium carbonate.

30

10. A carburizing material comprising a mixture of previously used carburizing material, crushed strongly coking material and an energizer.

In testimony whereof, I have hereunto 35  
subscribed my name this 13 day of June,  
1917.

HUGH RODMAN.

Witnesses:

R. L. KENT,  
ANNA CLOHERTY.